

## UNITED STATES PATENT OFFICE

2,431,435

## PRODUCTION OF CRINKLED CELLULOSE ESTER FILAMENTS

William Ivan Taylor, Spaldon, near Derby, England, assignor to British Celanese Limited, London W. 1, England, a company of Great Britain

No Drawing. Application February 18, 1944,  
Serial No. 522,968. In Great Britain March 24,  
1943

5 Claims. (Cl. 18—47.5)

1

This invention is concerned with improvements in the production of crinkled cellulose ester filaments and particularly in the production of artificial wool having a basis of cellulose acetate or other organic derivative of cellulose.

Wool is greatly valued as a textile fibre by reason of the heat-retaining qualities and soft handle of fabrics made thereof. These qualities appear to be associated in no small measure with the crinkly nature of the wool fibres. This has led to the production of crinkly artificial fibres and these "artificial wools" do exhibit in considerable measure the foregoing desirable qualities of wool. It is very desirable that such artificial wools should have crinkle and soft handle in a high degree and it is equally important that these qualities should not be adversely affected when fabrics, garments and other articles made from the artificial wools are subjected to normal wear or laundering. It is further desirable that such articles should revert to their original dimensions and shapes after distortion. Again, such artificial wools should be capable of being dyed evenly, as otherwise their value for many purposes is greatly diminished.

It has now been found that an artificial wool which exhibits in very high degree indeed the above-mentioned properties desirable in an artificial wool can be obtained by subjecting to the action of hot aqueous media filaments which have been made by a particular method from a solution of an organic derivative of cellulose, particularly of cellulose acetate.

According to the present invention, artificial filaments capable of yielding an improved artificial wool are obtained by extruding a solution of an organic derivative of cellulose in a volatile solvent through a spinning jet into a cell through which a current of evaporative medium is passed, said solution having a viscosity not exceeding 50 when determined as described below and, as it enters the spinning jet, being at a temperature below the boiling point of the solvent at atmospheric pressure.

The viscosity of the spinning solution or "dope" is measured by determining the time in second for a steel ball weighing 0.7 gm. and having a diameter of  $\frac{3}{2}$ " to fall through 3" of the solution at 25° C. The number of seconds is taken as representing the viscosity. Preferably a solution having a viscosity of from 25 to 30 is used in the production of artificial filaments by the process of the present invention.

The viscosity of the solution is dependent on the concentration of cellulose derivative in the solution. It is also dependent on the viscosity of

2

the cellulose derivative which is usually measured by determining the rate of flow of a fairly dilute solution of the derivative through an Ostwald viscometer. For instance, viscosities of the acetone-soluble cellulose acetates mentioned in this specification were determined by comparing the rate of flow of a 6% solution of the acetate in acetone at 25° C. with that of glycerine taken as 100. Thus a solution which has a rate of flow such that the level of the solution drops from the upper mark to the lower in 20 seconds, whereas glycerine requires 100 seconds under the same conditions, contains an acetate having a viscosity of 20.

15 The process of the present invention is of particular value in the production of filaments capable of yielding artificial wool from solutions of lower fatty acid esters of cellulose, e. g., cellulose acetate, cellulose propionate, cellulose butyrate, 20 cellulose acetate-propionate and cellulose acetate-butyrate and in the production of artificial wool from these filaments. Of the lower fatty acid esters, cellulose acetate is the most important and the invention will therefore be particularly described in relation to the production of artificial filaments having a basis of this ester and of artificial wool therefrom.

The normal method of producing cellulose acetate filaments consists in spinning a solution 30 of cellulose acetate in acetone, containing about 25% by weight of cellulose acetate, at a temperature of 70–80° C. into a counter-current of air which is at a similar temperature. The production of cellulose acetate filaments by the process

35 of the present invention involves the spinning of a solution of cellulose acetate at a low temperature into an evaporative medium which is preferably also at a low temperature, employing a spinning solution or "dope" which has a low viscosity. 40 Filaments may thus be obtained which crinkle extremely readily, evenly, and to an exceptionally high degree under the influence of hot aqueous media, compared with filaments obtained from the same cellulose acetate under ordinary conditions. If, however, one or more of the foregoing spinning conditions are not observed, the resulting filaments yield less satisfactory artificial wool upon subjection to hot aqueous treatments.

As an indication of spinning conditions which 50 have been found suitable, it may be stated that, when using a solution in acetone of ordinary acetone-soluble cellulose acetate having a viscosity of between 10 and 20, a dope temperature between 40–45° C., an air temperature in the cell from about 30–40° C. down to the dew point, and

a cellulose acetate concentration of about 18-22% are usually suitable. It will be noted that the temperatures employed are below the boiling point of the solvent present in the dope and that the low concentration of cellulose acetate will result in a dope of low viscosity. The lower the temperature, particularly of the dope, and the lower the cellulose acetate concentration, the more readily in general are the filaments crinkled by hot aqueous media and the better is the artificial wool produced. The temperatures and concentration cannot, however, be reduced below a certain minimum, which varies with the viscosity of the cellulose acetate and the other spinning conditions, if stable spinning is to be obtained. Usually, temperatures should be of the order of those given above. However, if it is desired to reduce the time required for the setting of the filaments the air temperature may be increased up to about the boiling point of the dope solvent, e. g., 55-60° C. when acetone is used. If an acetate of high viscosity, for example 50, 80, 100, 200 or more, is used, then there is a corresponding decrease in the minimum dope concentration which can be employed without reducing the dope viscosity below that necessary for stable spinning.

The use of low temperatures and low dope concentrations increases the length of time required to effect setting of the extruded filaments and it is, therefore, in general necessary either to spin at a slower speed than that usually employed in the dry-spinning of cellulose acetate filaments or to increase the length of the path of the materials through the evaporative medium. Both these expedients may, of course, be adopted in order to effect setting of the materials. For example, spinning speeds of 100 to 150 or 200 metres per minute may be employed, instead of the speeds of 300 or 500 metres per minute or even more used in the commercial production of ordinary cellulose acetate filaments, and the path of the materials through the evaporative medium may be increased to 15, 25 or 30 feet or more. Provided that the filaments pass for a substantial distance, e. g., 10, 12 or 15 feet, through an evaporative medium at a relatively low temperature, so that the major proportion of the solvent has been evaporated and the cross-sectional form of the filaments is established, they may then pass through a hotter evaporative medium, at a temperature of, e. g., 60-80° C., in order to accelerate removal of any residual solvent. In such cases it is convenient to use a co-current of evaporative medium so as to prevent overheating of the evaporative medium into which the filaments first pass.

As indicated above, the most important factors in the production of the filaments according to the present invention are the use of a low dope concentration and of a low dope temperature. A further factor which is of importance is the concentration of solvent in the evaporative medium, particularly in the region of the jet. In general, it is found that it is desirable to have a higher concentration of solvent in this region than is the practice in the production of ordinary cellulose acetate yarns. For example, using a counter-current of air the volume ratio of air to dope may be adjusted so that the outgoing air contains 2% of acetone by volume instead of about 1-1.5%, which is a normal figure, thus increasing the acetone concentration in the region of the jet.

In order to produce the artificial wool the fila-

ments, either in continuous form or after conversion into staple fibre, are subjected to treatment with a hot aqueous medium. Preferably they are heated for about 2-4 hours in a solution of a wetting agent, e. g., a soap solution containing, for instance, 0.5 to 1% of soap at a temperature from 90-100° C., though wet steam or hot water alone may be employed. The treatment should be carried out so that the filaments are free to contract and crinkle.

Continuous filaments are preferably assembled into yarns, with or without twisting, at the time of spinning and the yarns are subjected to the hot aqueous treatment in hank form. When the filaments have been crinkled the yarns may be twisted or further twisted and if a heavier denier yarn is required a number of ends may be assembled and then twisted either with the same twist or with a reverse twist to that employed with the single ends. Usually it is preferable to use a reverse twist. The method of twisting and whether one or a number of ends are employed will, however, depend upon the nature of the yarns which it is desired to produce. For instance, if artificial wool yarn of heavy denier is required it is generally desirable to form it from a number of ends whereas a yarn of light denier may consist of only one end.

Yarns may also be obtained according to the present invention by subjecting the assemblies of continuous filaments after spinning to a process of twisting, setting the twist and removing the twist such as is described in U. S. Patents S. Nos. 2,089,198, 2,089,199 and 2,111,211—preferably prior to treatment with a hot aqueous medium. Filaments in the form of staple fibres may be spun into yarns either prior to or after crinkling by a hot aqueous treatment. Again, yarns may be employed in the pile of a pile fabric and the pile then crinkled by a hot aqueous treatment.

The following example is given to illustrate the production of wool-like yarns by the process of the present invention.

#### Example

A 21.5% solution of a cellulose acetate, having a viscosity of about 16, in a liquid medium consisting of 95% acetone and 5% water was spun through twin jets into a cell and taken up at about 180 metres per minute. The viscosity of the spinning solution, determined as described above, was 25 and its temperature at the exit from the candle, i. e. on entering the jets, was 42°. The spinning conditions were such that each end had a total denier of about 340. The extruded filaments were passed for about 15 feet through a current of air at a temperature of 30-35° C. and the two ends were then taken up together outside the cell on cap spinning bobbins which inserted an S twist of 0.4 turns per inch into the yarn. The yarn was then hanked and the hanks heated for about 4 hours at a temperature of 90-100° C. in a 0.5% soap solution, after which they were washed and dried. The twist in the yarn was then increased to about 3 turns per inch after which three ends were doubled together with a Z-twist of 3 turns per inch. A yarn was thus obtained which dyed evenly and after finishing was very suitable for a hand-knitting yarn.

As has already been stated, yarns may be obtained by the process of the present invention which have outstanding properties as artificial wool and indeed in some respects are better than wool itself. For example, the permanent stretch of a sample of all-wool hand knitting yarn, after

stretching in dry and wet states under certain conditions, was respectively 26% and 29.5%, while that of the cellulose acetate yarn obtained as described above was only 4.8% and 16.0% respectively under the same conditions. It was also stronger than the wool sample when wet. As a consequence of the above improved properties articles can be made from the yarns which are much more resistant to stretching than articles made of pure wool and which thus keep their shape much better. For example, jumpers knitted from artificial wool obtained as described above retained their shape and showed negligible shrinkage after they had been washed ten times.

While, as indicated above, yarns produced by the spinning process described in the present application are particularly valuable for conversion into artificial wool by treatment with hot aqueous liquids they are also of value for other purposes. They may, for example, be employed without further treatment for the production of fabrics and other articles. Special effects may be produced by treating articles containing such yarns, either alone or combined with other yarns, with hot aqueous media so as to crinkle them.

The process of the present invention has been described particularly with reference to the production of filaments and artificial wool from cellulose acetate but, as has already been stated, it is also applicable to the production of filaments and artificial wool from other organic derivatives of cellulose. As indicated above the lower the dope concentration and the lower the temperatures of the dope and the evaporative medium, the better in general are the filaments produced for conversion into artificial wool, provided that stable spinning can be obtained. The temperatures employed will depend largely upon the nature of the solvent medium used and in general it is desirable that they should be substantially below its boiling point at atmospheric pressure, e. g., at least 10° C. lower. The dope concentrations which are suitable will depend on the cellulose derivative and solvent employed, but they will in any case be such as to yield a solution having a viscosity below 50 and will preferably be low enough to yield one of 25-30.

Having described my invention, what I desire to secure by Letters Patent is:

1. Process for the production of textile materials, which comprises forming continuous artificial filaments by extruding a solution of a lower fatty acid ester of cellulose in acetone through a spinning jet into a cell through which a current of air at a temperature at least 10° C. below the boiling point of acetone is passed, said solution having a viscosity between 25 and 50 when determined as hereinbefore described and, as it enters the spinning jet, being at a temperature below the boiling point of the solvent at atmospheric pressure.

2. Process for the production of textile materials, which comprises forming continuous artificial filaments by extruding a solution of cellulose

lose acetate in acetone through a spinning jet into a cell through which a current of air at a temperature at least 10° C. below the boiling point of acetone is passed, said solution having a viscosity between 25 and 50 when determined as hereinbefore described and, as it enters the spinning jet, being at a temperature between 40 and 45° C.

3. Process for the production of textile materials, which comprises forming continuous artificial filaments by extruding a solution of acetone-soluble cellulose acetate in acetone through a spinning jet into a cell through which a current of air at a temperature at least 10° C. below the boiling point of acetone is passed, said solution having a viscosity between 25 and 50 when determined as hereinbefore described and, as it enters the spinning jet, being at a temperature below the boiling point of the solvent at atmospheric pressure, and the rate of flow of air through the cell being such that on issuing from the cell it contains at least 2% of acetone by volume.

4. Process for the production of textile materials, which comprises forming continuous artificial filaments by extruding a solution of cellulose acetate in acetone through a spinning jet into a cell through which a current of evaporative medium at a temperature at least 10° C. below the boiling point of acetone is passed, said solution having a viscosity between 25 and 30 when determined as hereinbefore described, and, as it enters the spinning jet, being at a temperature between 40 and 45° C.

5. Process for the production of artificial wool, which comprises forming continuous artificial filaments by extruding a solution of cellulose acetate in acetone through a spinning jet into a cell through which a current of evaporative medium at a temperature at least 10° C. below the boiling point of acetone is passed, said solution having a viscosity between 25 and 50 when determined as hereinbefore described and, as it enters the spinning jet, being at a temperature between 40 and 45° C., and then treating the artificial filaments with a dilute aqueous solution of a wetting agent at a temperature of at least 90° C. but not exceeding the boiling point of the solution at atmospheric pressure until crinkling is effected.

WILLIAM IVAN TAYLOR.

#### REFERENCES CITED

The following references are of record in the file of this patent:

#### UNITED STATES PATENTS

| Number    | Name           | Date           |
|-----------|----------------|----------------|
| 1,554,801 | Dreyfus et al. | Sept. 22, 1925 |
| 1,930,230 | Dreyfus et al. | Oct. 10, 1933  |
| 1,952,877 | Mancini        | Mar. 27, 1934  |
| 2,072,102 | Dreyfus et al. | Mar. 2, 1937   |
| 2,217,113 | Hardy          | Oct. 8, 1940   |
| 2,232,012 | Rooney et al.  | Feb. 18, 1941  |